

E. F. COLLINS & J. A. CAPP,  
PROCESS OF SHERARDIZING,  
APPLICATION FILED MAR. 17, 1914.

1,169,529.

Patented Jan. 25, 1916.



Witnesses:

*Julian O'poner*  
*Benjamin B. Hesse*

Inventors:

John A. Capp,  
Edgar F. Collins,  
by *Albert. Dan*  
Their Attorney.

# UNITED STATES PATENT OFFICE.

EDGAR F. COLLINS AND JOHN A. CAPP, OF SCHENECTADY, NEW YORK, ASSIGNEES TO  
GENERAL ELECTRIC COMPANY, A CORPORATION OF NEW YORK.

## PROCESS OF SHERARDIZING.

1,169,528.

Specification of Letters Patent. Patented Jan. 25, 1916.

Application filed March 17, 1914. Serial No. 325,431.

To all whom it may concern:

Be it known that we, EDGAR F. COLLINS and JOHN A. CAPP, citizens of the United States, residing at Schenectady, county of Schenectady, State of New York, have invented certain new and useful Improvements in Processes of Sherardizing, of which the following is a specification.

Our present invention relates to the art 10 of coating metals with zinc, known generally as sherardizing. The sherardizing process appears to have been originated and developed by Sherard Cowper-Coles, and is set forth in his U. S. Patent #701,298, June 15, 1902. According to this process the articles to be sherardized are packed in a closed drum containing ordinary zinc dust of commerce, and the drum is then placed in a furnace and submitted to the action of heat 20 for a length of time necessary to produce a coating of zinc upon the articles. The zinc dust of commerce is a by-product obtained through the practice of metallurgical processes for obtaining metallic zinc and consists 25 of minute particles of metallic zinc coated or associated with zinc oxid. The zinc content in the form of metallic zinc may vary anywhere from 20% to 90% while at the same time there may be various impurities 30 present such as lead, silica, and iron oxid. Instead of employing this zinc dust of commerce in its natural state, it is the practice in many cases, with a view to obtaining a better coating of zinc on the finished articles, 35 to dilute the zinc dust by the addition of fine sand, the amount of sand added forming a very large proportion of the resulting mixture. In some cases the amount of sand added was so proportioned that the amount 40 of metallic zinc present in the mixture was not greater than about 25%.

Temperatures employed in carrying out the process appear to vary widely in practice. The temperature recommended by the patentee in the patent above referred to, is that corresponding to "the dull red heat of iron" which is probably in the neighborhood of 450° C., or higher. The temperatures employed by various users of the process, as appears from published and other data, are in general very materially lower than this figure, and in some cases as low as 400° F. corresponding to 204° C.

The sherardizing process as heretofore practised produced a deposit of coating

which in general was of a light gray color, varying in some cases from a bright silvery color to a dull gray. From our researches it appears that the light color of the coating is largely due to the presence therein of 60 zinc oxid, the lighter the coating the more oxid being present.

In the prior practice of the sherardizing process the drums containing the articles to be sherardized, packed in the zinc dust, 65 were fired or heated in furnaces of various types, as for example, oil or gas fuel furnaces. The temperatures of such furnaces are difficult to control except within wide limits. Not only does the temperature of 70 such a furnace vary greatly from time to time but also the temperatures are frequently very widely different at a given instant at different points in the contents of the drum.

The result of the sherardizing process as thus carried out has been the production of zinc coated or sherardized articles which when submitted to severe weather and other conditions were found to be not satisfactorily 80 protected from rust, which of course is one of the main objects of the sherardized coating. In some cases the sherardized articles, consisting of malleable iron castings or the like, have rusted within a few days when 85 exposed to the salt air of the seashore or to similar conditions. The sherardizing process has therefore not been used so extensively as it might be nor has it always given satisfaction when used.

We have discovered as a result of our investigations that a greatly improved quality of sherardized coating may be produced provided a certain correlation be observed 90 between the composition of the zinc dust and the temperature at which the articles are sherardized. With respect to the composition of the zinc dust, this should be as free from impurities as possible, and especially free from lead. Very small quantities of silica or iron oxid do not appear to be deleterious. The zinc dust should be rich in metallic zinc. The percentage of metallic zinc should preferably be about 85% but may vary from 80% as a minimum to 92%. 100 As a maximum. The remainder of the mixture, except for slight impurities, should consist of zinc oxid. The ordinary zinc dust of commerce is ordinarily too low in metallic zinc and we therefore prefer to use zinc 105 110

powder, which is an artificially produced atomized metallic zinc, containing only a very small percentage of zinc oxide or impurities. When this zinc powder is first used in the sherardizing drums a blank run is first made, that is to say, without any articles being packed in the drums for sherardizing, whereby the oxygen present in the air in the drum combines with zinc to produce zinc oxid. Upon conclusion of this heat treatment, the zinc dust is submitted to chemical analysis and if its content of metallic zinc is found to fall within the limits of 80% to 92%, it is then ready for use. Should the zinc content be too low then the proper proportion of metallic zinc in the form of powder is added and if the zinc content is too high then the charge is reheated to produce further oxidation. As the content of metallic zinc in the charge is reduced by repetitions of the sherardizing operation, it is necessary to make up for this by regularly adding zinc powder between runs in quantity sufficient to keep the metallic zinc content within the limits indicated. This quantity is determined after careful chemical analysis of the charge which analyses should be made at frequent intervals.

The temperature which we employ for sherardizing with the zinc dust mixture of the richness indicated, we find should lie within relatively small limits, the lower limit of temperature being 350° C. and the upper limit 375° C., though a very slight variation either way may be tolerated. With such a close temperature range within which to carry on the sherardizing, it is evident that a very special type of furnace is necessary so that the temperature may be raised uniformly throughout the charge to the operating temperature and maintained very closely the same throughout the entire charge. Any material variations of the operating temperature from the range of temperature which we have indicated will result in an inferior product, and for this reason it has been found to be practically impossible to carry out our process with ordinary types of gas or oil heated furnaces heretofore used for sherardizing.

The furnace which we have found best adapted to the carrying out of our process is a furnace making use of electrically produced heat. The heating coils or conductors may be located at proper points in relation to the charge so that the entire charge may be heated throughout very closely to the same temperature.

In the drawings we have illustrated, by way of example, a furnace suitable for use in carrying out our improved process.

In general the furnace consists of a box of suitable construction for containing the charge, mounted on trunnions so that it may be rotated, and provided with electric heat-

ing units on all sides exposed to the charge so that all portions of the charge may be raised to the same desired temperature and there maintained. The details of construction may of course vary widely.

In the drawings one form of furnace suitable for the purpose is indicated, in some respects diagrammatically, certain portions being cut away or shown in section so as more clearly to indicate the construction.

The box which directly contains the charge is in this instance made of cast iron and is indicated in the drawings in section at 1, and is provided with a cast iron cover similarly indicated at 2. Upon each of the five sides of the box, and upon the cover, heating units made of strips of sheet metal or other suitable material are applied as indicated for example at 3. These heating units are held in place by metal clamping plates such as 4, 85 and are insulated both from the box and the clamping plates by sheets of insulating material such as 5, 6 consisting of built-up sheets of mica or the like. The heating units on the cover of the box are similarly insulated from the cover 2 and the corresponding clamping plate 7. The box proper, as well as its cover, is provided with an outer shell or casing of sheet metal. The casing for the box proper is indicated at 8 and for the cover the 95 casing is indicated at 9. These casings are so applied as to provide a considerable space between the casing and the members which they inclose, and in this space heat insulating material such as asbestos, mineral wool or the like is placed as indicated, for example at 10 and 11.

The cover of the furnace box is held in place by any suitable means, such for example as clamping bars 12 and 13, the ends 105 of which project through slots in lugs 14 formed integral with the box 1 and projecting up through appropriate openings in the cover. Clamping screws indicated at 16 screw down upon bosses or lugs 17 which 110 are formed integral with the cover plate 2 and project up through openings in the sheet iron casing 9. Ring bolts 18 are provided whereby the cover may be lifted off when the clamping devices have been removed.

The entire box is mounted upon trunnions, one of which is indicated at 19, these trunnions being carried by pillow blocks or other bearings 20. Some suitable gearing is provided, such for example as a worm and worm 120 wheel 21 and 22, for setting the box into slow rotation. Collector rings 23, 24, and 25 mounted on a projecting shaft 26, and provided with suitable current conveying brushes, not shown, serve to convey current 125 to the heating units in the box. Three collector rings are shown in this case so that connections may be made to the heating units whereby the heating units may be connected in series or in multiple, in order to provide 130

for current adjustment. Thus, upon starting up the apparatus, the heating units may be connected in two sections in multiple with each other, and when the desired temperature is reached the connections may be changed to series, further adjustment being taken care of by appropriate external regulators.

In order that the temperature of the charge may be properly controlled, thermometers are placed in tubes such as 27 extending through the walls of the furnace box into close proximity to the charge. A well known form of angle thermometer is indicated at 28.

It is important, in carrying out our process, that the temperature of the charge in the sherardizing drum or furnace should be raised as quickly as possible to the working or operating temperature for the reason that the sherardized coating which is deposited at temperatures lower than this working temperature is inferior, and hence the shorter the time taken in reaching the working temperature the less proportion this inferior coating will bear to the total. For this purpose, in starting the sherardizing operation, the electric current applied to the heating coils is made very much greater at first than after the desired temperature of the charge has been reached. When this desired temperature has been reached, the heating current is cut down until only just enough energy is supplied to make up for the heat losses. When the desired working temperature of 350° C. to 375° C. has been attained the electric current is controlled so that the temperature of the charge will remain within the limits noted. The temperature of the charge is preferably ascertained by means of thermometers inserted into the charge through openings in the sherardizing box or drum as already described. The readings of these thermometers will obviously vary somewhat but all ought to lie within the range above noted.

The length of time for carrying out the sherardizing operation according to our process varies somewhat according to the thickness of coating desired but runs anywhere from 6 to 12 hours.

If during the sherardizing operation the temperature is allowed to rise materially above 375° C., we find that the deposit or coating becomes coarse and crystalline, whereas if the temperature is allowed to fall materially below the lower limit of 350° C., the coating becomes relatively soft and porous. In both cases the coating is decidedly inferior. Moreover, good results will not be secured even within the temperature range we have indicated unless the composition of the mixture is such that the metallic zinc content is within the range of 80 to 92%. If there is more metallic zinc present than that represented by the upper limit of ap-

proximately 92%, the mass of powder becomes sticky and pasty so that the proper coating does not take place, while if the mixture has a less percentage of zinc than about 80% then the sherardized coating is of less definitely metallic character being therefore like the soft and spongy coat applied at too low temperature, and incapable of withstanding corrosive action.

The sherardized coating produced according to our process wherein the composition of the zinc dust and the temperature of sherardizing are correlated as above described, is never lumpy or uneven in thickness as frequently happens when the temperature and composition of the zinc mixture are not controlled as we have set forth. On the contrary the coating is so smooth, even and uniform in thickness, that by proper time allowance a coating of any desired thickness may be applied with great exactness. This makes it possible to sherardize articles like nuts and bolts so that the threads fit exactly without, as has heretofore been the case, requiring the smoothing action of taps or dies to smooth off the threads, a proper undercutting of the threads having been made to compensate for the subsequent application of the coating. Also, our improved sherardized coating is far superior in resisting corrosion to the sherardized coatings heretofore produced. One distinguishing characteristic of sherardized coatings made in accordance with our process is that of color. For example, malleable iron castings, when they have been submitted to treatment according to our process, have a color almost black, or which might perhaps be described as a very dark and dingy gray. The color is entirely distinct from that characteristic of the ordinary sherardizing which is a light, and in some cases is a very light, silver gray. In the case of a malleable iron or similar casting treated by our process, the article after removal from the sherardizing drum or furnace does not appear greatly different in color from that which it possessed before treatment. In fact, to the unpractised eye, our improved sherardizing does not appear to have changed the color of the article in a very marked degree. Upon careful cleaning of the sherardized article, however, by removing any adherent particles of dust by rubbing, the sherardized coating appears to be not so much black as bluish, which is the characteristic color of pure zinc metal. The dark color of the sherardized metal produced by our process is perhaps explainable by the fact that it contains such a large percentage of pure zinc and so little zinc oxid. This is indicated by the specific gravity of the coating which, in the case of that applied according to our method, is exceedingly high and in the neighborhood of 6.5 to 6.75 as compared with the specific gravity of 1.15

pure zinc which is 7.15. Sherardized coatings of lighter color such as heretofore produced, have a specific gravity much lower and averaging perhaps in the neighborhood of 3.5.

Our improved sherardizing coating is far superior to the ordinary coating in its capacity to resist corroding influences. An ordinary test for measuring the value of zinc coatings in this respect, known as the Preece test, consists in dipping the article in a solution of copper sulfate, washing and drying, and then repeating the operation, until the coating breaks down. With this test applied, coatings made by our improved process are able to withstand eight to twelve dips whereas the prior sherardized coatings were able to withstand only one to five dips under the same conditions. We have found, however, that the Preece test is not in all respects a true indication of the capacity of the coating to resist ordinary corroding influences such as sea water, sea air, etc., and we have devised a test wherein the length of time during which the article is capable of resisting certain corroding influences is more nearly a true measure of the lasting qualities of the coating in ordinary use. We provide a box or closed space in which by means of an atomizer operated by compressed air a light spray is produced from a strong brine, or salt solution. The articles to be tested are placed on a grating in this salt spray. Under this treatment, we have found that ordinary sherardizing lasts only a few hours, at most only two or three days, whereas our improved sherardizing will last indefinitely, without breaking down, and showing rust.

10 The mechanical properties of sherardized coatings made by our process are also noteworthy. Articles so coated may be bent, swaged or otherwise deformed, at ordinary room temperatures, without injury to the coating. The coating does not crack or flake off, as has been found to be the case

with sherardized coatings as heretofore applied, but remains an integral part of the article.

What we claim as new and desire to secure by Letters Patent of the United States, is:

1. The method of sherardizing which consists in submitting the articles to be sherardized to the action of zinc dust or powder containing not less than 80% nor more than 92% metallic zinc, the remainder being mainly zinc oxid while maintained at a working temperature which does not fall below 350° C. nor rise above 375° C. 60

2. The method of sherardizing which consists in so correlating the composition of the zinc dust or powder, and the working temperature of treatment that the percentage of zinc in the dust lies within the limits of about 80% to 92%, while the temperature of treatment lies within the range between about 350° C. and 375° C. 65

3. The improvement in the art of sherardizing which consists in maintaining the sherardizing temperature so that it does not exceed 375° C. or fall below 350° C. while the zinc dust is maintained substantially free from impurities and with a percentage of metallic zinc within the limits of 80% to 92%. 70

4. A metallic article having a sherardized zinc coating capable of resisting rusting influences indefinitely, said coating having a specific gravity of not less than 6.5, a color approximating that of an ordinary malleable iron casting and a union with the metallic article such that the coating does not crack, flake or peel off when the article is deformed by bending, swaging or the like. 80

In witness whereof, we have hereunto set our hands this 16th day of March, 1914.

EDGAR F. COLLINS.  
JOHN A. CAPP.

Witnesses:

BENJAMIN B. HULL,  
HELEN ORFORD.